

1

3,518,172  
PROCESS FOR THE ELECTROLYSIS OF  
ALUMINUM CHLORIDE

Gilbert S. Layne and James O. Huml, Midland, Mich., and Richard Dale Smith, Madison, Conn., assignors to The Dow Chemical Company, Midland, Mich., a corporation of Delaware  
No Drawing. Filed Feb. 24, 1967, Ser. No. 618,335  
Int. Cl. C22d 3/12

U.S. CL. 204—67

8 Claims

### ABSTRACT OF THE DISCLOSURE

The molten salt electrolysis of aluminum chloride to produce aluminum and chlorine is improved by employing as at least one bath component an alkali or alkaline earth fluoride as a vapor pressure control agent. The effective volatilization temperature of aluminum chloride is thereby significantly increased.

### BACKGROUND OF THE INVENTION

Aluminum is commercially produced by the Hall-Heroult process in which  $Al_2O_3$  dissolved in a molten cryolite bath is electrolyzed. In addition to the electrical energy required, the process requires the consumption of about 0.5 pound of carbon or graphite electrode per pound of aluminum produced. Oxides of carbon are consequently produced as valueless by-products.

Since the early days of aluminum technology, inventors have been seeking ways to electrolyze  $AlCl_3$ . Although slightly more theoretical electrical energy is required, the electrolysis of  $AlCl_3$  does not require the consumption of carbon electrodes and, indeed, produces a valuable by-product, chlorine gas. However, the practical use of  $AlCl_3$  to produce aluminum and chlorine has been thwarted by a number of problems. For instance, the vapor pressure of  $AlCl_3$  gas is high over melts at temperatures of greater than 660° C., the melting point of aluminum, such melts tend to creep and the electrical conductivity of melts containing  $AlCl_3$  is usually poor.

### SUMMARY OF THE INVENTION

This invention relates to an improved process for the electrolysis of aluminum chloride and more particularly relates to a process for the electrolysis of aluminum chloride in a fused salt bath with improved physical and electrochemical properties.

It is an object of this invention to provide an improved method whereby aluminum chloride may be retained in a fused salt electrolytic bath. It is a further object of this invention to provide an improved process for the electrolysis of aluminum chloride. These and other objects and advantages of the process will be readily appreciated and become better understood by reference to the following detailed description.

It has now been discovered that a molten halide salt bath containing aluminum chloride may be electrolyzed above the normal volatilization temperature of aluminum chloride by the addition to such molten salt bath of certain alkali or alkaline earth metal fluorides as vapor pressure control agents. Mixtures containing these vapor pressure control agents must be molten or produce a molten mixture when contacted with aluminum chloride. The vapor pressure control agents are added in an amount sufficient to decrease the vapor pressure of the resultant molten salt bath to the desired level at electrolysis temperature. As used herein, the term "halide" refers to chloride or fluoride.

2

### BRIEF DESCRIPTION OF PREFERRED EMBODIMENTS

As vapor pressure control agents, lithium fluoride, sodium fluoride, potassium fluoride, magnesium fluoride, calcium fluoride, strontium fluoride, and barium fluoride have been found to be effective but particular advantage has been found in the use of calcium fluoride. These alkali and alkaline earth metal fluorides may be used as vapor pressure control agents alone, mixed with one another, or as mixed salts with aluminum fluoride. Likewise, such fluorides may be used in combination with other standard fused salt bath components such as sodium chloride or calcium chloride. The proportion of such fluoride to be added to a fused salt bath of aluminum chloride will depend on the desired vapor pressure of the molten salt mixture at the selected temperature of electrolysis. In general, however, a concentration of  $AlCl_3$  in the fused salt bath of up to about 20 percent is preferred. The proportion of fluoride ion required as a vapor control agent is at least 2 fluoride ions to 1 Al ion, preferably an atom ratio of fluoride ion to aluminum ion of from about 2:1 to about 10:1.

There are other factors to be considered in the optimization of the bath composition for  $AlCl_3$  electrolysis. It is usually desirable, for instance, to maximize the electrical conductivity of the bath and to minimize the fluorine content of the anode chlorine gas. It has been found beneficial to maintain a chloride to fluoride ion ratio in the bath of at least 2:1, preferably from about 2:1 to about 10:1. This insures that the fluorine content of the chlorine gas is at a low level. The selection of the cations required to fulfill the above conditions plus any further dilution of these baths with metal halides should be made on the basis of improvement in electrical conductivity and other physical properties of the molten salt bath.

To illustrate, a favorable composition for  $AlCl_3$  electrolysis is 8 mole percent  $AlCl_3$ , 25 mole percent  $CaF_2$ , and 67 mole percent  $CaCl_2$ . This system, which melts below 700° C. has, at 975° C., a vapor pressure of about 7 mm. Hg and an electrical conductivity of about 2.6 reciprocal ohm-cm. These values compare favorably with those found in the Hall-Heroult  $Al_2O_3$ -cryolite cell and are superior to those melts previously proposed for  $AlCl_3$  electrolysis.

Once the desired quantity of alkali or alkaline earth metal fluoride has been added to the fused salt bath and electrolysis started, aluminum chloride may be continuously added to produce aluminum and gaseous chlorine. While the mechanism of this process is not known with certainty, it is thought to proceed according to the following equations wherein M is an alkali or alkaline earth metal fluoride as defined above and X is the valence of such alkali or alkaline earth metal fluoride.



The net effect of the reaction therefore is



As the alkali or alkaline earth metal fluoride vapor pressure control agent is continuously regenerated in situ, its concentration remains relatively constant. No additional fluoride need be added except to replace mechanical losses and the like, and substantially no fluoride ion increase occurs which necessitates replacement of the bath.

Electrolysis of the fused salt bath to produce aluminum and chlorine may be conducted in a standard manner. The process can be batch or preferably continuous as taught in the patent art.

The following examples are provided as a more detailed description of the various embodiments of the invention but are not to be construed as limiting the scope thereof.

Example 1

A 1309 gm. portion of  $\text{Na}_3\text{AlF}_6$  was heated in a graphite crucible to 1000° C. in an argon atmosphere. Gaseous aluminum chloride was then added below the surface of the melt by passing it through a graphite tube immersed in the molten  $\text{Na}_3\text{AlF}_6$ . During the addition of  $\text{AlCl}_3$  to the molten salt bath, no  $\text{AlCl}_3$  fumes were noticeable above the melt. After a total of 209 gm. of  $\text{AlCl}_3$  had been added, the bath was cooled and analyzed by X-ray diffraction. Analysis showed about 40 weight percent  $\text{AlF}_3$ , 40 weight percent  $\text{NaCl}$  and about 20 weight percent  $\text{Na}_5\text{Al}_3\text{F}_{14}$ .

Example 2

The following experiment was conducted to illustrate the exchange of halide ions:

To a graphite crucible in an inert atmosphere was added 56 gm. of  $\text{AlF}_3$  and 58.5 gm. of  $\text{NaCl}$ . The salt mixture was then melted by heating to 900° C. Electrolysis was conducted at a potential of 3.0 volts using a centrally located graphite rod as the anode and the crucible as the cathode. Chlorine gas and aluminum metal were produced but no  $\text{AlCl}_3$  vapors were observed over the bath.

Example 3

In the same manner as Example 1,  $\text{AlCl}_3$  was added to a molten bath of  $\text{CaCl}_2$  and  $\text{CaF}_2$  at 900° C. to form a bath composition of 25 mole percent  $\text{CaF}_2$ , 65 mole percent  $\text{CaCl}_2$  and 10 mole percent  $\text{AlCl}_3$ . At 900° C. the vapor pressure of  $\text{AlCl}_3$  over the resultant melt was found to be less than 10 mm. of mercury and the electrical conductivity was found to be  $2.4 \text{ ohm}^{-1} \text{ cm.}^{-1}$ . Electrolysis of the melt produced chlorine and aluminum. Continued electrolysis was conducted by continuously adding gaseous  $\text{AlCl}_3$  to melt.

Example 4

In an inert atmosphere, gaseous  $\text{AlCl}_3$  was added to a pure  $\text{CaF}_2$  melt contained in a graphite crucible by introduction of the gas beneath the melt surface. Additions of  $\text{AlCl}_3$  began at a temperature of 1450° C. and were completed at 900° C. The final melt contained 25 mole percent  $\text{AlCl}_3$  and 75 mole percent  $\text{CaF}_2$ . The melt had a freezing point of about 675° C. and a vapor pressure of about 11 mm. Hg at 900° C. A decomposition potential of 2.1 volts was observed during a brief period of electrolysis and the products of electrolysis were identified as aluminum and chlorine.

Various modifications can be made in the present invention without departing from the spirit or scope thereof for it is understood that we limit ourselves only as defined in the appended claims.

We claim:

- 5 1. In a process for the electrolysis of aluminum chloride in a fused halide salt bath at a temperature above the normal volatilization temperature of said aluminum chloride, the improvement which comprises employing, as at least one molten component of said fused salt bath, an alkali or alkaline earth metal fluoride vapor pressure control agent in an amount sufficient to increases the effective volatilization temperature of the aluminum chloride to above the temperature of electrolysis of the melt and maintaining in said fused salt bath an ion ratio of fluoride ion to aluminum ion of at least 2 to 1.
- 10 2. The process of claim 1 wherein the vapor pressure control agent is at least one member selected from the group consisting of  $\text{LiF}$ ,  $\text{NaF}$ ,  $\text{KF}$ ,  $\text{MgF}_2$ ,  $\text{CaF}_2$ ,  $\text{SrF}_2$  and  $\text{BaF}_2$ .
- 15 3. The process of claim 1 wherein the vapor pressure control agent is calcium fluoride.
- 20 4. The process of claim 1 wherein the vapor pressure control agent is  $\text{Na}_3\text{AlF}_6$ .
- 25 5. The process of claim 1 wherein the ion ratio of chloride ion to fluoride ion is at least 2 to 1.
- 30 6. The process of claim 1 wherein the ion ratio of fluoride ion to aluminum ion is from about 2:1 to about 10:1 and wherein the ion ratio of chloride ion to fluoride ion is from about 2:1 to about 10:1.
- 35 7. The process of claim 1 wherein the fused salt bath consists essentially of from about 2 to about 12 mole percent  $\text{AlCl}_3$ , from about 19 to about 29 mole percent  $\text{CaF}_2$  and the remainder being  $\text{CaCl}_2$ .
- 40 8. The process of claim 1 wherein the fused salt bath consists essentially of about 8 mole percent  $\text{AlCl}_3$ , about 25 mole percent  $\text{CaF}_2$  and about 67 mole percent  $\text{CaCl}_2$ .

References Cited

UNITED STATES PATENTS

- |           |         |        |        |
|-----------|---------|--------|--------|
| 2,919,234 | 12/1959 | Slatin | 204—67 |
| 3,103,472 | 9/1963  | Slatin | 204—67 |

FOREIGN PATENTS

- |         |        |                |
|---------|--------|----------------|
| 648,337 | 1/1951 | Great Britain. |
| 687,758 | 2/1953 | Great Britain. |
| 757,908 | 9/1956 | Great Britain. |

50 JOHN H. MACK, Primary Examiner

DONALD R. VALENTINE, Assistant Examiner